

Patented Apr. 26, 1949

2,468,458

# UNITED STATES PATENT OFFICE

2,468,458

## METHOD OF MANUFACTURING RESISTANCE ELEMENTS

Adriaan Abraham Padmos and Evert Johannes Willem Verwey, Eindhoven, Netherlands, assignors, by mesne assignments, to Hartford National Bank and Trust Company, Hartford, Conn., as trustee

No Drawing. Application May 3, 1946, Serial No. 667,106. In the Netherlands April 29, 1942

Section 1, Public Law 690, August 8, 1946  
Patent expires April 29, 1962

4 Claims. (Cl. 25—157)

1

In a copending application for a U. S. Patent Serial No. 668,471, filed May 9, 1946, a method is disclosed with the aid of which it is possible to manufacture sintered resistance bodies which have a high resistance value and a low temperature coefficient of the resistance and which consist of an insulating mass of magnesia in which particles of reduced electrically conducting titanium oxide are dispersed in a quantity of 3% at the most.

According to this method, a mixture of magnesia and titanium oxide is sintered at a temperature beyond 1700° C., preferably of from 1800 to 2000° C., in a reducing gas stream whose content of oxygen with respect to the hydrogen present therein amounts to at least 0.003% by volume and for the rest is exactly adjusted in connection with the desired resistance value.

For wholesale manufacture this method can be further improved in various respects.

In the method described in the copending application, the content of oxygen of the reducing gases which surround the resistance bodies during the sintering operation is particularly important in connection with the obtainment of the desired resistance value. Now it has been found that this content of oxygen can be regulated not only by the choice of the composition of the gas introduced but also by adjusting the speed of flow. The correct speed of flow may be ascertained for each individual case by a preliminary test. This method of adjustment is particularly important in wholesale manufacture since in this case comparatively large numbers of resistances are treated simultaneously and therefore the amount of oxygen taken up in the gas during the reduction may have an appreciable influence on the reducing character thereof.

For carrying the invention into effect use may be made with particular advantage of the embodiment described in the copending application wherein the starting-point is formed by partly reduced titanium oxide or by corresponding mixtures of titanium dioxide and titanium because in this case a smaller amount of oxygen is set free and consequently the content of oxygen of the gas surrounding the resistance bodies can be regulated more easily by means of the speed of flow. Now it has been found that such a favourable influence is exerted not only by titanium in the starting mixture but also by silicon and carbon. Moreover, these additions bring about a slight displacement of the temperature coefficient of the resistance in the positive direction, which is desirable for some applications.

2

Since in general an increase of the content of reduced titanium oxide in the resistance material results in that the temperature coefficient becomes more negative, we obtain the further advantage, more particularly with the use of the above-mentioned additions, that the total of the content of titanium oxide can be slightly increased, for example to about 4%, for it is thus possible to obtain resistances which have a still lower specific resistance than that obtained in accordance with the method described in the copending application whilst the low temperature coefficient and the other favourable properties are retained.

15 The invention will hereinafter be explained more fully with reference to one example.

Magnesia which has been preliminarily heated to 1300—1400° C., is ground, jointly with approximately 4% by weight of rutile and 1 1/4% by weight 20 of carbon with alcohol, during 8 hours in a ball-mill whereupon, with the use of nitrocellulose as a binder, the material is pressed into rods which are dried. Subsequently, these rods are sintered during about 6 minutes in a gas stream 25 consisting of a mixture of about 90% by volume of nitrogen and 10% by volume of hydrogen, this gas being purified by causing it to pass over finely divided Cu present on infusorial earth and heated to 300° C. and dried with the aid of solid 30 KOH, liquid oxygen and P<sub>2</sub>O<sub>5</sub>. The heating takes place with the aid of a molybdenum tube heated by an electric current to 1800—1900° C., said tube having a length of 30 cms. and an internal diameter of 8 mms. If the speed of the flowing gas 35 is adjusted to 16 litres per minute we obtain resistances which, when having a length of 18 mms. and a diameter of 1.35 mms., have at room temperature a resistance value of about 1.5×10<sup>4</sup> ohms. At a temperature of 300° C. the resistance value is approximately 70% of the value at room 40 temperature.

What we claim is:

1. A method of manufacturing resistance elements, comprising the steps of sintering a mixture of magnesium and titanium oxides at a temperature greater than about 1700° C. in a reducing gas stream containing hydrogen and oxygen in the amount of at least 0.003% by volume of the hydrogen, and controlling the amount of oxygen in said reducing gas stream by adjusting the flow of said reducing gas over said sintered mixture.

2. A method of manufacturing resistance elements comprising the steps of sintering a mixture of magnesium and titanium oxides contain-

3

ing a small addition of an element selected from the group carbon and silicon at a temperature greater than about 1700° C. in a reducing gas stream containing hydrogen and oxygen in the amount of at least 0.003% by volume of the hydrogen, and controlling the amount of oxygen in said gas stream by adjusting the flow of said reducing gas over said sintered mixture.

3. A method of manufacturing resistance elements, comprising the steps of sintering a mixture containing magnesium oxide, approximately 4% by weight of titanium oxide, and a small addition of an element selected from the group carbon and silicon at a temperature greater than about 1700° C. in a reducing gas stream containing hydrogen and oxygen in the amount of at least 0.003% by volume of the hydrogen, and controlling the amount of oxygen in said reducing gas stream by adjusting the flow of said reducing gas over said sintered mixture.

4. A method of manufacturing resistance elements, comprising the steps of sintering a mix-

ture of magnesium oxide, approximately 4% by weight of titanium oxide, and approximately 1 1/4% by weight of carbon in a gas stream comprising approximately 90% by volume of nitrogen and approximately 10% by volume of hydrogen at a temperature between approximately 1800° C. and 1900° C., and adjusting the flow of gas over said mixture to about 16 liters per minute.

10 ADRIAAN ABRAHAM PADMOS.  
EVERT JOHANNES WILLEM VERWEY.

## REFERENCES CITED

15 The following references are of record in the file of this patent:

## UNITED STATES PATENTS

|    | Number    | Name      | Date          |
|----|-----------|-----------|---------------|
|    | 1,992,482 | Heuer     | Feb. 26, 1935 |
| 20 | 2,021,520 | Reichmann | Nov. 19, 1935 |
|    | 2,095,982 | Heany     | Oct. 19, 1937 |
|    | 2,316,228 | Erdmann   | Apr. 13, 1943 |